

# United States Patent

Jansen et al.

[15] 3,688,151

[45] Aug. 29, 1972

[54] **DEVICE HAVING AN ELECTRIC DISCHARGE TUBE COMPRISING A FIELD EMISSION CATHODE, AND DISCHARGE TUBE DESTINED FOR SUCH A DEVICE**

[72] Inventors: Constant Gijsbertus Johannes Jansen; Klaas Compaan; Albertus Venema, all of Emmasingel, Eindhoven, Netherlands

[73] Assignee: U.S. Philips Corporation, New York, N.Y.

[22] Filed: Sept. 14, 1970

[21] Appl. No.: 71,806

[30] **Foreign Application Priority Data**

Sept. 18, 1969 Netherlands.....6914205

[52] U.S. Cl. ....313/348, 313/268, 313/337

[51] Int. Cl. ....H01j 1/46, H01j 1/52, H01j 17/04

[58] Field of Search.....313/348, 268, 337

[56]

## References Cited

### UNITED STATES PATENTS

|           |         |               |            |
|-----------|---------|---------------|------------|
| 3,363,136 | 1/1968  | Pakswer ..... | 313/268    |
| 1,618,499 | 2/1927  | White .....   | 313/268 UX |
| 3,154,711 | 10/1964 | Beggs.....    | 313/337 X  |

### FOREIGN PATENTS OR APPLICATIONS

|           |        |              |         |
|-----------|--------|--------------|---------|
| 1,359,344 | 3/1964 | France.....  | 313/268 |
| 746,016   | 1943   | Germany..... | 313/268 |

Primary Examiner—David Schonberg

Assistant Examiner—Toby H. Kusmer

Attorney—Frank R. Trifari

[57]

## ABSTRACT

In a cold cathode consisting of a layer of aluminum oxide between a plate and a grid, the aluminum oxide is formed on aluminum as a porous oxide layer. The meshes of the grid are so fine that the grid is attracted against the oxide due to the voltage difference with the plate.

4 Claims, 2 Drawing Figures



PATENTED AUG 29 1972

3,688,151



Fig.1



Fig.2

INVENTORS  
CONSTANT G.J. JANSEN  
KLAAS COMPAAN  
ALBERTUS VENEMA  
BY

Jan C. K. van der Linde  
AGENT

**DEVICE HAVING AN ELECTRIC DISCHARGE  
TUBE COMPRISING A FIELD EMISSION  
CATHODE, AND DISCHARGE TUBE DESTINED  
FOR SUCH A DEVICE**

The invention relates to a device having an electric discharge tube comprising a field emission cathode consisting of a layer of aluminum oxide on which a conductive metal layer is present on one side and a metal grid which has a positive potential relative to the conductive metal layer is present on the other side. The invention furthermore relates to an electric discharge tube destined for such a device.

The aluminum oxide in the cathode described in the German patent specification 746,016 consists of a comparatively thick sintered mass. The metal layer is provided on the aluminum oxide as a metallization. The metal grid is preferably pressed in the aluminum oxide layer. The emission current is assumed to consist of electrons which move from the interior of the aluminum oxide to the apertures in the metal grid and there either emanate themselves, or liberate secondary electrons from the edges of the grid. Once the emission has started, it is not necessary to apply an external potential difference between the two electrodes at the aluminum oxide, since as a result of the emission the potential difference is automatically maintained. However, this applies only if the cathode goes on supplying current. In so far as it is known, the cathode described has not resulted in practical applications and data on the emission density to be achieved with the cathode and the value of the applied voltages are not known either.

From French patent specification 1,359,344 a cold cathode is known which consists of an aluminum plate on which a layer of aluminum oxide with a thickness of from 100 to 300 AU is formed by vapor-deposition or by anodic oxidation. On this layer is present a layer of a metal, such as gold, platinum or palladium, obtained by vapor-deposition, which layer in turn is covered with a thick porous layer of magnesium oxide which has likewise been obtained by vapor-deposition. The thickness of this layer is in the order of 50  $\mu\text{m}$ . The cathode requires a voltage of approximately 10 volts across the layer of aluminum oxide.

In the cathode known from French patent specification 844,616 a layer of a material having a low work function, an alkali metal or alkaline earth metal is present between a thin aluminum oxide layer and the support. The aluminum oxide is covered by a gauze, or by a very thin metal layer which is permeable to electrons. With a voltage of approximately 1 volt across the aluminum oxide, currents in the order of 1 A could be reached with a value of the cathode which is not stated. In order to stimulate the emission, the cathode can be slightly heated or be exposed to infrared radiation. The field emission occurring in the cathode is said to be obtained as a result of all these measures at field strengths of  $10^4$  V/cm a factor 100 to 1,000 lower than normal. Practical applications of said cathode are not known.

It is the object of the invention to provide a device of the type mentioned in the preamble having a simple and rigid construction.

According to the invention, in a device having an electric discharge tube comprising a field emission cathode consisting of a layer of aluminum oxide on which a conductive metal layer is present on one side

and a metal grid which has a positive potential relative to the conductive metal layer is present on the other side, the aluminum oxide layer consists of a porous oxide layer having a thickness of from a few  $\mu\text{m}$  to a few tens  $\mu\text{m}$  formed on an aluminum support by anodic oxidation.

Such porous aluminum oxide layers which have long been known already (see A.J. Decker and W.Ch. van Geel, Philips Res. 2, 313-319, 1947) have a substantially hexagonal structure in which cavities and pillar-like particles of aluminum oxide, both with a diameter of a few hundred of AU directed at right angles to the surface, seem to alternate. The cavities and pillars of oxide are separated from the underlying aluminum by a closed layer of aluminum oxide the thickness of which expressed in tens of AU is approximately equal to the voltage expressed in volts applied in the electrolytic formation of the layer. As an electrolyte in the formation of the layer is used oxalic acid or another acid in which exclusively the formation of aluminum oxide occurs.

In connection with the thickness of the porous oxide layer, the required potential difference across the layer is in the order of 50 volts or higher. However, this involves that if the metal grid has a sufficiently low thickness, wire thickness 50  $\mu\text{m}$  and less, the gauze is attracted, throughout the surface of the cathode, by the electrostatic force. The advantage of this with respect to a more rigid grid of thicker wires which is held only by mechanical force is that it better engages the surface of the cathode, which promotes the uniformity of the emission across the surface.

In order that the invention may be readily carried into effect, it will now be described in greater detail, by way of example, with reference to the accompanying drawing, in which

FIG. 1 is a diagrammatic representation on a strongly exaggerated scale of the electrode system of an electric discharge tube according to the invention with the associated electric connections and

FIG. 2 shows a few current-voltage characteristics.

Reference numeral 1 in FIG. 1 denotes a strip of aluminum which has been bent at right angles and has an upper surface area of 0.3 sq.cm. A porous oxide layer 2, thickness 5  $\mu\text{m}$ , in which cavities are present at right angles to the surface, is present on the aluminum, the cavities and the intermediate oxide having transverse dimensions of from 200 to 500 AU. Below said layer is a thin layer of aluminum oxide having a thickness of approximately 100 AU. A copper gauze 3, mesh width 40  $\mu\text{m}$ , wire thickness 7  $\mu\text{m}$ , is present on the aluminum oxide 2. The anode is constituted by a nickel plate 4 at a distance of 2 mm from the gauze 3. The electric connection of the aluminum plate, the gauze and the nickel anode are denoted by 5, 6 and 7. The current limiting resistors 8 and 9, respectively, each 1  $\text{M}\Omega$ , are included in the connection leads to 5 and 7.

In FIG. 2 the voltage difference between the connection terminals 6 and 7 in volts is plotted on the horizontal axis, and the electron current in  $\mu\text{A}$  which flows to the anode 4 is plotted on the vertical axis, curve A applying to the case in which the voltage between 5 and 6 is 120 volts and curve B applying to the case in which said voltage is 180 volts. The currents in said circuit are 2.0 and 12.5  $\mu\text{A}$  respectively.

What is claimed is:

1. A device having an electric discharge tube comprising a field emission cathode consisting of a layer of aluminum oxide on which a conductive metal layer is present on one side and on which a metal grid which has a positive potential relative to the conductive metal layer is present on the other side, said aluminum oxide layer consisting of a porous oxide layer formed on an aluminum support by anodic oxidation.

2. A device as claimed in claim 1, wherein the potential difference across the aluminum oxide layer is so large that the metal grid is attracted against the aluminum oxide layer by the electrostatic force.

3. A device as claimed in claim 2, wherein the poten-

tial difference across the aluminum oxide layer is more than 50 volts.

4. An electric discharge tube destined for a device as claimed in claim 1, wherein the porous aluminum oxide layer has a hexagonal structure in which cavities at right angles to the surface alternate with intermediate material, both with transverse dimensions in the order of magnitude of hundreds of AU and the cavities and the intermediate material are separated from the underlying aluminum by a closed layer of aluminum oxide having a thickness in the order of magnitude of hundreds of A-units.

\* \* \* \* \*

15

20

25

30

35

40

45

50

55

60

65